

1

2,732,799

## METHODS FOR INSOLUBILIZING COATING COMPOSITIONS

John Harris Haslam, Newport, Del., assignor to E. I. du Pont de Nemours and Company, Wilmington, Del., a 5 corporation of Delaware

No Drawing. Application March 17, 1950,  
Serial No. 150,350.

15 Claims. (Cl. 101—416)

This invention relates to imprinting and coating operations, and more particularly to novel methods for rendering ink impressions upon various surfaces substantially non-smearing in nature.

Printing presses usually operate at high speeds; the more rapid the rate at which printing matter can be produced, naturally the greater the output in a given period of time or the shorter the time required for a given output. For example, newsprint is generally passed through presses at about 1600 ft. per minute; and magazines and other periodicals which have a definite publication deadline are printed on high speed presses also. The greatest problem in achieving rapid printing lies in the printing inks. In order to wet paper or textile, glass or metal, or the like, and thus effect a relatively lasting impression thereon, ink must initially be fluid. However, such fluidity is disadvantageous in that, if the printed surface contacts another surface while the ink is still wet, the ink will smear and become blurred or blotted. Further, the ink, once thoroughly dry, should become insoluble, so that it will not smear if the printed surface should later become wetted. It is thus vital for clear impressions that the ink be dry and non-tacky before the printed surface is contacted, and that it be permanently insolubilized. There is a continuous search by the trade for methods whereby inks may be dried and rendered permanent more and more quickly.

In the case of newsprint, the porosity of the paper employed allows the ink to be quickly absorbed therein. It is because of this that the above-mentioned high printing speed of 1600 ft. per minute is possible. In the case of magazines and other periodicals which use a less porous paper, and in the case of printing on metals, glass, various fabrics and other less pervious surfaces, absorption is of little or no aid and possible printing speeds are materially less. One method generally employed to dry or set inks applied to such materials is simple evaporation of the solvent, often with heat. At best, this is time-consuming and costly. Magazine print is passed over an open flame at temperatures as high as 650° C., and the solvent is thus quickly flash-vaporized. However, even by this shorter procedure, the highest usually obtainable press speed is about 900 ft. per minute; furthermore, the intense heat serves to weaken and generally degrade the fibers of the paper, resulting in costly web breaks and shutdowns. Another commercial method is to dissolve a solid resin in a solvent and then precipitate it from such solution by addition of a second material in which it is insoluble. Thus, a resin vehicle may be dissolved in ethylene glycol and mixed with a pigment to form a conventional ink. This ink may then be impressed on a printing surface. If the impression is brought into contact with water (generally added as steam), the vehicle will be precipitated from the glycol solution and thereby insolubilized. In such a system the second solvent must be miscible with the first, but the vehicle must be insoluble in a mixture of the two. Such requirements seriously restrict the number of systems possible; and the rate of insolubilization, even with satisfactory solvent systems, is relatively slow, no really fast drying method utilizing this principle having been developed.

As will be evident, the problem of insolubilizing or rapidly setting inks employed in various printing ap-

2

plications is one of major importance, and a great need exists for a novel procedure whereby such inks may be more rapidly dried, the possible speed of printing consequently increased, and printing costs advantageously lessened. It is among the objects of this invention, therefore, to meet this problem and to provide novel procedures for accomplishing such objects. A particular object is to provide novel means for rendering ink impressions upon a printing surface substantially non-smearing in character. A specific object is to effect the rapid and thorough setting or drying of an ink following its application to a printing surface. Other objects and advantages of my invention will be apparent from the ensuing description thereof.

These objects are attained in this invention which broadly comprises accelerating the drying of a pigmented coating composition containing a polymerizable, organic polyhydroxy compound, by subjecting said composition to reaction with an organic ester of a fourth group metal selected from titanium and zirconium.

In a more specific and preferred embodiment, the invention comprises substantially instantaneously drying an ink composition applied to a paper or other surface by subjecting said composition (containing a colorant and as a vehicle a polymerizable, organic polyhydric compound having a molecular weight of at least 500 and more than one free, reactive hydroxyl group) to insolubilization through reaction with a titanium or zirconium ortho ester of a primary aliphatic alcohol containing from 1-8 carbon atoms.

Since the invention is particularly useful (though not limited) to the quick drying of ink type coating compositions used to produce characters in writing or printing upon a paper or other suitable surface, it will be described in its application to such adaptation and particularly in printing inks. These are employed for use in the usual type, copper plates, etc., and comprise syrupy, non-smudging, so-called lithographic varnish compositions exhibiting a suitable consistency and adapted to be readily transferred from conventional ink rolls to the type and from the type to the paper or other surface to which the ink is to be applied. They consist of a suitable linseed oil and rosin or other oil vehicle in which lamp black or any other suitable inorganic or organic colorant, such as conventional white or colored pigments or dyestuffs, or mixtures thereof to obtain various shades or tints, are incorporated or dispersed. Examples of utilizable colorants include titanium dioxide, zinc sulfide, lithopone, blue to green phthalocyanines, lead chromate, vermillion, Venetian red, cobalt blue, indigo, iron blue, Miloni blue, chrome greens, azo maroons, etc.

The coating or ink composition used, to be effectively useful in accordance with the invention, must contain, either as a vehicle or as a component part of the composition, a polyhydroxy compound such as glycol, glycerol, pentaerythritol, castor oil, nitrocellulose, etc. Polyhydroxy compounds having a molecular weight of at least 500 and containing more than one free hydroxyl group, adapted to react with a titanium or zirconium ester to induce quick drying and insolubilization of the composition following its application to a surface are preferred for use. Among examples of these compounds, those of nitrocellulose, phthalic anhydride-glycerol alkyd resins (either modified or unmodified), bisphenol-epichlorhydrin resins, pentaerythritol alkyds, etc., can be mentioned.

The polyhydroxy compound, like the composition vehicle, should be in the liquid phase. It itself may be a liquid or can be present as a solute. If a solid or semi-solid, it must be capable of being dissolved in conventional organic solvents in accordance with customary printing practice. If a liquid, it should polymerize to a solid, or if a soluble solid, it should polymerize to an

insoluble form. It can be incorporated directly in the vehicle or composition to form a component part of each; or, if preferred, the vehicle can consist entirely of the compound or be composed of suitable mixtures of polyhydroxy compounds. Thus, where a solid or semi-solid form is used, resort can be advantageously had to a polyhydroxy compound type solvent, such as glycerin or glycol, etc., to effect dissolution and subsequent use in such solvent. In such instance the metal ester will react with both the vehicle and solvent to produce an insoluble ink film comprising a polymer of vehicle plus solvent plus ester. If desired, more than one vehicle can be used in a given composition, as may various mixtures and combinations of utilizable vehicles and solvents.

The polyhydroxy compound-containing ink or like coating composition, upon being conventionally impressed upon a surface as by transfer from, for example, an ink roll to a paper, textile, glass, metal, etc., is immediately subjected to contact with, preferably, a stoichiometric quantity of a contemplated metal ester. Those found to be of particular value for use in the invention comprise the organic esters of titanium or zirconium. Surprisingly, all metal esters are not satisfactory for use herein since silicon esters, for example, prove of little or no value for use. It appears that the desired insolubilization and rapid set of polyhydroxy vehicles is attained only with esters of metals which have a coordination number higher than their valence. Thus, zirconium and titanium have coordination numbers of 6, while silicon has a coordination number of 4. In practice, essentially any titanium or zirconium ester (or alcoholate) or mixtures of such compounds can be used in the invention. They are readily formed by replacing a hydroxy hydrogen of an alcohol with titanium or zirconium. One useful method of preparation comprises reacting an alcohol with a halide, preferably the chloride, of titanium or zirconium in the presence of ammonia, and in accordance with the procedures of U. S. Patent No. 2,187,821. Because of their availability and commercial attractiveness, use is preferred of titanium or zirconium ortho esters of alcohols having from 1-8 carbon atoms in their primary chains; e. g., methyl, butyl, secondary butyl, propyl, isopropyl, tertiary-butyl, ethyl, amyl, and like esters, substituted or unsubstituted. Representative esters of such compounds include ethyl titanate, butyl titanate, octyl titanate, phenyl titanate, phenyl ethyl titanate, and cyclohexyl titanate, etc., as well as the zirconates of these representative titanates.

As in the case of the polyhydroxy vehicle, the ester may be employed in the form of a liquid or solution, or, if a solid, it may be dissolved in a suitable anhydrous solvent prior to use. In the latter instance, a solvent which also tends to insolubilize the particular polyhydroxy vehicle present is especially satisfactory, giving a combined and accentuated setting effect. Such contact of the ester with the coating composition can, for example, be effected by superimposing the ester upon the ink or other coating impression through overprinting, rolling or spraying, or by immediately subjecting the printing surface to a vaporous atmosphere of the ester while an elevated temperature condition prevails over such coated surface. In the latter instance, any alcohol or like by-products which form are readily removed as vapors.

In the interaction between the ester and organic compound, the latter is substantially instantaneously polymerized to render the ink or coating insoluble in either water or oils. The insolubilization occurring within one second or less, depending upon the particular polyhydroxy compound and ester utilized, results in a non-tacky print even before solvent evaporation to obviate the necessity of employing open-flame vaporization or other solvent removal methods and enable resort to a much less complex and generally more rapid printing operation. Additionally, the print, when dry, will not "set off" from the paper or other surface to which it is applied.

Although not definitely established, it appears that the reaction between the polyhydroxy compound and ester can be represented by the following equation:



10 in which R represents an alkyl, alkenyl, aryl, alkaryl, or arylalkyl grouping, x is at least 2 and preferably at least 3, Y is a polyfunctional organic radical, and Z is an integer greater than 1. The reaction shown is between a titanium ester of a monohydroxy organic compound, e. g., an alcohol and a polyhydroxy compound which may be represented by nitrocellulose or partially-hydrolyzed polyvinyl acetate. The reaction may of course proceed even further, and there may be various modifications and other chemical compounds formed. While polymerization and consequent insolubility can be achieved with practically any polyhydroxy vehicle, proper selection to fit the particular objective is recommended. For instance, glycerol may be reacted with a titanium or zirconium ester and will set rapidly but optimum results are not achieved in certain instances since the product tends to flake off of non-porous surfaces so that a relatively permanent impression upon such surfaces may not be obtained. On the other hand, a phthalic anhydride-glycerol resin of low molecular weight, though also utilizable and providing satisfactory binder action, tends to set up slowly in such applications and hence is not preferred for use where the highest setting speed is desired or required. Accordingly, the high-molecular-weight polyhydroxy organic compounds are more suitable for general usage on all types of surfaces. The various hydroxyl groups may be primary, secondary, or in any other positions; such compounds may be so-called "resins," partially-polymerized materials, monomers, dimers, or the like.

40 To a clearer understanding of the invention, the following examples, which are merely in illustration but not in limitation of such invention, are given:

#### Example I

45 10 parts by weight of a 30% by weight solution of nitrocellulose in n-butyl acetate were mulled after preparation with one part of lampblack. The resulting ink was then impressed upon paper by means of a rubber stamp. Meanwhile, butyl zirconate was dissolved in 50 toluene to provide a 50% by weight solution. Immediately after stamping the paper with the ink, the zirconium ester solution was applied thereover by means of a rubber roller. Immediately following such application, "setting" of the ink was tested by the simple expedient of rubbing the impression with the hand. It was found that within one second after the ester treatment the ink was completely dry and non-smearing, even though the experimenter's hand was moist and rather oily during the test. In a comparable experiment but in which ester treatment 55 was not resorted to, smearing occurred after the lapse of 120 seconds' time.

#### Example II

An alkyd resin made from undehydrated castor oil, 65 containing free hydroxyl groups from both unesterified glycerine and ricinoleic acid, was dissolved in xylol to provide a non-volatile content in the solution of 59.7%. 10 parts by weight of this solution were intimately mixed with 0.5 part of lampblack, following which the resulting 70 ink was printed upon a paper surface. Isopropyl titanate was vaporized by heating to a temperature of 232° C., and the resulting vapors were then reacted with the ink by directly contacting the printed surface with the evolved vapors. It was found that the ester treatment thus 75 effected permanently insolubilized the ink within one

second, in contrast to a 500-second period for insolubilization, where ester treatment was not used.

*Example III*

A soybean oil-modified alkyd resin, wherein the source of hydroxyl groups was unesterified or excess glycerin, was dissolved in xylol to provide a 49.2% by weight solution as an ink vehicle. 0.7 part by weight of lampblack was incorporated in 10 parts of this resin solution to provide an ink composition. Tertiary-butyl titanate (itself a liquid) was applied to a printing surface by means of a roller. Immediately after such application, the prepared ink was superimposed on such surface by conventional overprinting. As a result, the rate of setting of the ink under these conditions was found to be extremely rapid, being markedly less than one second.

*Example IV*

An ink was prepared by incorporating 0.3 part by weight of lampblack in 10 parts by weight of a 64.4% solution of a castor oil-modified alkyd resin in xylol. (This alkyd had a higher percentage of oil modification than the alkyd of Example II, but a lower free hydroxyl content.) An impression made by this ink on a printing surface was then insolubilized in about one second when sprayed with a toluene solution of n-amyl zirconate.

*Example V*

A 64.7% by weight solution in mineral spirits of a pentaerythritol alkyd resin (the free hydroxyl groups of which were of the primary alcohol type) was prepared, following which 10 parts by weight of this solution were thoroughly mixed with 0.13 part of lampblack to form an ink. This ink was printed upon a paper surface, the resulting print being then immediately sprayed with liquid n-propyl titanate. The ink impression was found to set in about 3 seconds, in contrast to a 500-second setting period when the titanium ester was not employed.

*Example VI*

An ink similar to those of the previous examples was prepared, by utilizing as the vehicle a 44.0% by weight solution of a bisphenol-epichlorhydrin resin in mineral spirits and .7 part by weight of lampblack. This ink was conventionally impressed upon a printing surface and was then contacted with vapors of isopropyl titanate. Reaction between the ester and the ink vehicle proceeded rapidly, the ink becoming polymerized and permanently insoluble in about 0.5 second. In a comparable experiment, but in which ester treatment to effect insolubilization was not resorted to, setting and drying of the ink did not take place until the lapse of 200 seconds.

*Example VII*

A dehydrated castor oil-modified resin was dissolved in xylol to give about a 50% solids content in the solution. A conventional ink was prepared with this material and used in printing. The resulting print was contacted with liquid ethyl titanate by rolling the latter across the surface. The ethyl titanate treatment caused the ink to set in between  $\frac{1}{4}$  and  $\frac{1}{2}$  second, in contrast to a 500-second period where ester treatment was not resorted to.

As shown in the examples, the invention possesses great flexibility both as to useful ingredients and the application of the ingredients or reactants. Its widest application is in the field of newspaper and periodical printing, but obviously it is commercially attractive for use in other fields and is applicable to coating compositions generally which contain polyhydroxy organic compounds in non-aqueous systems such as exist in paints, inks, varnishes, finishes, etc., or other coatings which may be applied to textiles, cellulose objects, plastics and other surfaces for decorating purposes and in which quick drying and insolubilization is desired. Insolubilization of such films may be had by the application of organic

titanates or zirconates such as ethyl, isopropyl, butyl or octyl titanates or zirconates, which, as already stated, can be applied in the fluid condition, i. e., as vapors or as liquids, to the printed or decorated surface.

The invention is useful in almost any type of printing and on widely different surfaces. The achievement of rapid set makes it particularly valuable for paper printing, where high speed presses are used, and for impressions on metals and glass where present drying methods are disadvantageously slow and clear print is difficult to obtain. It is also valuable for impressing designs and printing upon textile and other fabric surfaces. In this field, also, potential rapid-setting is a desired advance in the art. The impressions resulting from my process are substantially non-smearing and insoluble, not only in water but also in oils and organic solvents. The disadvantage of present paper inks is often that oil from the finger or hand will cause the ink to smudge, and a disadvantage of fabric inks is that they are not often wholly stable in the presence of solvents used in dry-cleaning. The ink films insolubilized by the present metal ester treatment will be found to overcome these disadvantages.

It will be seen from the above that many interrelated factors are to be considered in operating the present process. Thus, the binding quality of the insolubilized vehicle and the rapidity of its setting or drying are interdependent with the particular vehicle and ester chosen. Also of importance are the temperatures employed, the particular methods of print application or transfer, the surface on which the ink impression is being made, etc. Additionally, consideration should be given to the relative proportions of ester and vehicle used. Obviously, if less than a stoichiometric quantity of ester is employed, incomplete reaction and incomplete or slower setting may occur. It sometimes happens, also, that excess ester tends to slow the setting rate. Hence, it may be hypothesized that such excess serves as a solvent for the supposedly insoluble product and hydrolysis proceeds more slowly, or that too many metal groups by mass action actually allow less polymerization and cross-linking. The viscosity of the vehicle may also be a factor in its setting properties. If the ink is relatively thick, the surface may react immediately when the ester contacts it, while the underneath or unexposed area may remain unaffected. Under any circumstances, the elevation of the temperature will be found to speed the reaction and the rate of set. The effect of relatively mild heat is probably not simply to evaporate the solvent, as for instance in the case of the extreme heat of the open-flame process, but rather also to accelerate the chemical reaction between the vehicle and the ester.

Many varied methods of applying the vehicle and the ester to the printing surface are possible. As indicated, the pigmented vehicle or ink is generally first impressed upon a surface by any known or desired process and the ester is then superimposed on the resulting ink impression; where feasible, it may alternatively be introduced to the surface in vaporous form. Although this described order of addition is generally preferred, such order may be reversed, if desired, whereby the metal ester is applied first to the surface and the vehicle then superimposed thereon. It is sometimes satisfactory and feasible, too, to employ the present process in conjunction with the prior art methods. Thus, the open-flame process for printing of paper can be used with my ester treatment, or the procedure of insolubilization with a second solvent can be resorted to. The combined effect of my treatment with present commercial methods will sometimes serve to achieve even greater printing press speeds, or a lower necessary temperature for flash-vaporization, rendering it possible to obtain a clear and acceptable print with a less expensive, lower-grade paper.

I claim as my invention:

1. A method for insolubilizing and rapidly setting a printing ink coating composition applied to a surface,

comprising reacting a polymerizable, polyhydroxy organic compound in said coating while in liquid condition with a stoichiometric amount of an organic ester of an aliphatic monohydric alcohol containing from 1-8 carbon atoms of a metal selected from the group consisting of titanium and zirconium in the presence of said coating.

2. A process for accelerating the drying of a color-imparting ink coating composition containing as an essential ingredient a polymerizable polyhydroxy organic compound in the liquid state which comprises contacting said coating in its applied state to a surface and reacting said compound with a stoichiometric quantity of an organic ester of an aliphatic monohydric alcohol containing from 1-8 carbon atoms of a metal selected from the group consisting of titanium and zirconium.

3. An improved process of insolubilizing a polyhydroxy compound-containing ink coating composition on a surface to which it is applied which comprises reacting said compound in liquid state with a stoichiometric amount of an organic ester of an aliphatic monohydric alcohol containing from 1-8 carbon atoms of titanium.

4. An improved process of insolubilizing a polyhydroxy compound-containing ink coating composition on a surface to which it is applied which comprises reacting said compound in liquid state with a stoichiometric amount of an organic zirconium ester of a monohydric alcohol containing from 1-8 carbon atoms.

5. A process for accelerating the drying of an ink composition which comprises applying a pigmented ink composition containing an organic polyhydroxy compound to a printing surface and reacting the resulting ink impression while in liquid state with a stoichiometric amount of an organic ester of an aliphatic monohydric alcohol containing from 1-8 carbon atoms of a metal selected from the group consisting of titanium and zirconium.

6. A process for producing substantially non-smearing ink impressions upon a surface which comprises applying to said surface an ink composition containing a colorant and a polymerizable polyhydroxy organic compound and prior to drying said composition polymerizing said compound in situ by reaction with a stoichiometric amount of an organic ester of an aliphatic monohydric alcohol containing from 1-8 carbon atoms of a metal selected from the group consisting of titanium and zirconium.

7. A process for quickly drying a printing ink which comprises applying a pigmented printing ink composition containing as an essential ingredient a polymerizable polyhydroxy organic compound having a molecular weight of at least about 500 to a printing surface, and thereupon reacting said compound while in liquid state with a stoichiometric amount of an organic metal ester of an aliphatic monohydric alcohol containing from one to eight carbon atoms selected from the group consisting of titanium and zirconium.

8. A process for drying and insolubilizing a printing ink which comprises impressing upon a printing surface a pigmented ink composition containing as a vehicle a polymerizable polyhydroxy organic compound having a molecular weight of at least about 500, and insolubilizing said compound while in liquid state upon said surface within one second by reacting it with a stoichiometric amount of a metal ester of a primary aliphatic alcohol containing from one to eight carbon atoms, said metal being selected from the group consisting of titanium and zirconium.

9. A process for drying and insolubilizing a printing ink which comprises impressing upon a printing surface a pigmented ink composition containing as a vehicle a polymerizable polyhydroxy organic compound having a molecular weight of at least about 500, and insolubilizing said compound while in liquid state upon said surface within one second by reacting it with a stoichiometric amount of isopropyl titanate.

10. A process for drying and insolubilizing a printing ink which comprises impressing upon a printing surface

a pigmented ink composition containing as a vehicle a polymerizable polyhydroxy organic compound having a molecular weight of at least about 500, and insolubilizing said compound while in liquid state upon said surface within one second by reacting it with a stoichiometric amount of isopropyl zirconate.

11. A process for drying and insolubilizing a printing ink which comprises impressing upon a printing surface a pigmented ink composition containing as a vehicle a polymerizable polyhydroxy organic compound having a molecular weight of at least about 500, and insolubilizing said compound while in liquid state upon said surface within one second by reacting it with a stoichiometric amount of ethyl titanate.

12. A process for drying and insolubilizing a printing ink which comprises impressing upon a printing surface a pigmented ink composition containing as a vehicle a polymerizable polyhydroxy organic compound having a molecular weight of at least about 500, and insolubilizing said compound while in liquid state upon said surface within one second by reacting it with a stoichiometric amount of butyl titanate.

13. A process for drying and insolubilizing a printing ink which comprises impressing upon a printing surface a pigmented ink composition containing nitrocellulose as a vehicle, and insolubilizing said ink composition in liquid state on said surface within one second by reacting the nitrocellulose with a stoichiometric amount of a titanium ester of a monohydric alcohol containing from 1-8 carbon atoms.

14. A process for drying and insolubilizing a printing ink which comprises impressing upon a printing surface a pigmented ink composition containing bisphenol-epichlorhydrin as a vehicle, and insolubilizing said ink in liquid state composition on said surface within one second by reacting the bisphenol-epichlorhydrin with a stoichiometric amount of a titanium ester of a monohydric alcohol containing from 1-8 carbon atoms.

15. A process for drying and insolubilizing a printing ink which comprises impressing upon a printing surface a pigmented ink composition containing castor oil as a vehicle, and insolubilizing said ink composition in liquid state on said surface within one second by reacting the castor oil with a stoichiometric amount of a titanium ester of a monohydric alcohol containing from 1-8 carbon atoms.

#### References Cited in the file of this patent

#### UNITED STATES PATENTS

|    |           |              |       |               |
|----|-----------|--------------|-------|---------------|
| 50 | 1,752,462 | Smith        | ----- | Apr. 1, 1930  |
|    | 1,900,603 | Coolidge     | ----- | Mar. 7, 1933  |
|    | 1,933,520 | Bruson       | ----- | Oct. 31, 1933 |
|    | 2,109,774 | Hooft        | ----- | Mar. 1, 1938  |
|    | 2,116,321 | Minich       | ----- | May 3, 1938   |
| 55 | 2,132,997 | Plechner     | ----- | Oct. 11, 1938 |
|    | 2,187,821 | Nelles       | ----- | Jan. 23, 1940 |
|    | 2,208,587 | Kienle       | ----- | July 23, 1940 |
|    | 2,258,718 | Rothrock     | ----- | Oct. 14, 1941 |
| 60 | 2,518,193 | Signaiga     | ----- | Aug. 8, 1950  |
|    | 2,518,607 | Erickson     | ----- | Aug. 15, 1950 |
|    | 2,528,850 | Thorp et al. | ----- | Nov. 7, 1950  |
|    | 2,613,162 | Chatfield    | ----- | Oct. 7, 1952  |

#### FOREIGN PATENTS

|    |         |               |       |               |
|----|---------|---------------|-------|---------------|
| 65 | 346,812 | Great Britain | ----- | Apr. 17, 1931 |
|    | 513,222 | Great Britain | ----- | Oct. 6, 1939  |

#### OTHER REFERENCES

- Ellis: *Printing Inks*. Published 1940 by Reinhold Publishing Co., N. Y. Only page 100 cited.
- Minich: *The Anionics of Driers*. Presented February 15, 1950. Published in *Official Digest*, July 1950, pp. 533 to 540. Only pp. 533 to 535 relied on.
- Minich: *The Anionics of Driers*. Previously cited. 75 Pages 536 and 537 added.